

## UNITED STATES PATENT OFFICE

2,221,257

## MAGNESIUM BASE ALLOY

John C. McDonald, Midland, Mich., assignor to  
The Dow Chemical Company, Midland, Mich., a  
corporation of Michigan

No Drawing. Application November 13, 1939,  
Serial No. 304,134

3 Claims. (Cl. 75—168)

The invention relates to magnesium base alloys. It more particularly concerns alloys of this nature having a high degree of formability coupled with other improved physical properties, 5 such as increased tensile and yield strengths.

Magnesium alloys are being widely used in various structural and mechanical arts where a light weight metal is highly desirable, such as for use in making castings, forgings, and the like. 10 However, the use of these alloys in the rolled form to make sheet metal articles requiring forming operations such as bending, drawing and the like has not progressed as rapidly due to the fact that in general alloys having good form- 15 ability, permitting relatively sharp bends to be made without the article developing external cracks, usually have inferior tensile and yield strengths.

It is accordingly the principal object of this 20 invention to provide a magnesium base alloy which may be made into rolled sheet or the like, possessing a high degree of ductility or formability together with high strength characteristics.

25 Other objects and advantages of the invention will be apparent as the description of the invention proceeds.

My invention resides in the discovery that a

acteristics, is manifest over the entire range of composition indicated, I have found that in general the preferred combination of properties, such as satisfactory ductility for forming operations together with high tensile and yield 5 strengths, is found in alloys containing from 0.5 to 4 per cent of silver, 6 to 12 per cent of cadmium, and from 0.5 to 4 per cent of zinc. In general the alloys containing the higher percentages of the alloying ingredients have higher 10 strength properties, making them very suitable for use in casting operations as well as forming operations.

The specific proportion of each alloying metal and the total amount of the added metals to be 15 employed in the new alloy depends upon the use for which the alloy is intended. In general it is preferable to employ an alloy containing more than about 75 per cent magnesium and less than 25 per cent of the total added metals.

The following table, which lists some of the 20 properties of rolled sheet metal made from my new alloy, as well as the properties of sheet metal made from related ternary alloys, illustrates the improvement in yield strength, tensile strength, 25 and ductility or formability, as represented by the per cent elongation increase, of my new alloy over that of the closely related alloys.

Table

| 30 | Nominal composition in percent<br>(remainder-magnesium) |     |     | Annealed |                                      |                                        | Cold rolled                          |                                      | 30                                     |    |
|----|---------------------------------------------------------|-----|-----|----------|--------------------------------------|----------------------------------------|--------------------------------------|--------------------------------------|----------------------------------------|----|
|    | 35                                                      | Ag  | Cd  | Zn       | Yield<br>strength in<br>lbs./sq. in. | Tensile<br>strength in<br>lbs./sq. in. | Percent<br>elongation<br>in 2 inches | Yield<br>strength in<br>lbs./sq. in. | Tensile<br>strength in<br>lbs./sq. in. |    |
|    |                                                         |     |     |          |                                      |                                        |                                      |                                      |                                        |    |
| 40 | 35                                                      | 0.8 | —   | 0.9      | 17,000                               | 32,000                                 | 17                                   | 32,000                               | 37,000                                 | 35 |
|    |                                                         | 0.9 | 4.8 | —        | 16,000                               | 31,000                                 | 15                                   | 28,000                               | 35,000                                 | 40 |
|    |                                                         | 0.9 | 5.0 | 0.9      | 18,000                               | 32,000                                 | 20                                   | 36,000                               | 42,000                                 | 45 |
|    |                                                         | 0.9 | 4.8 | —        | 16,000                               | 31,000                                 | 15                                   | 28,000                               | 35,000                                 | 50 |
|    |                                                         | 0.8 | 5.1 | 4.7      | 31,000                               | 41,000                                 | 14                                   | 40,000                               | 46,000                                 | 55 |
| 45 | 40                                                      | 4.0 | —   | 1.0      | 19,000                               | 33,000                                 | 15                                   | 28,000                               | 36,000                                 | 30 |
|    |                                                         | 2.9 | 5.0 | 0.9      | 17,000                               | 33,000                                 | 20                                   | 35,000                               | 42,000                                 | 35 |
|    |                                                         | 4.0 | —   | 1.0      | 19,000                               | 33,000                                 | 15                                   | 28,000                               | 36,000                                 | 40 |
|    |                                                         | 5.8 | 5.4 | 1.0      | 26,000                               | 38,000                                 | 16                                   | 40,000                               | 48,000                                 | 45 |
|    |                                                         | 0.8 | —   | 0.9      | 17,000                               | 32,000                                 | 17                                   | 32,000                               | 37,000                                 | 50 |
| 50 | 45                                                      | 8.7 | —   | 0.9      | 18,000                               | 33,000                                 | 17                                   | 30,000                               | 38,000                                 | 30 |
|    |                                                         | 0.9 | 8.4 | —        | 16,000                               | 31,000                                 | 15                                   | 28,000                               | 35,000                                 | 35 |
|    |                                                         | 0.9 | 9.0 | 0.9      | 21,000                               | 35,000                                 | 24                                   | 34,000                               | 41,000                                 | 40 |
|    |                                                         | 0.9 | 8.4 | —        | 16,000                               | 31,000                                 | 15                                   | 28,000                               | 35,000                                 | 45 |
|    |                                                         | 0.8 | 9.4 | 5.5      | 27,000                               | 40,000                                 | 16                                   | 41,000                               | 48,000                                 | 50 |

magnesium base alloy composed of from 0.5 to 50 10 percent of silver, from 1 to 15 per cent of cadmium, and from 0.1 to 10 per cent of zinc, the balance being substantially all magnesium, is endowed with the aforementioned properties. While the property of improved formability or 55 ductility, associated with high strength char-

The properties listed in the above table under the section headed by the term "annealed" were 50 obtained by first rolling the alloys at a temperature between about 500° to 600° F., and thereafter annealing them at various temperatures through a temperature range of from 400° to 800° F. The properties selected for the table were those of 55

the annealed specimens which exhibited the maximum elongation. The properties listed under the section headed "cold rolled" were obtained by subjecting specimens of the alloys which had been hot rolled at a temperature of from 500° to 600° F. to additional rolling in the cold state to bring about a total reduction in thickness of from 2 to 10 per cent. The properties selected for the table were those of the cold rolled specimens which showed the greatest tensile and yield strengths, while having at least a 1 per cent elongation in 2 inches.

By comparison of the properties listed in the above table, it will be observed that the combined properties of my new quaternary alloy are superior to those of the parent ternary alloys having similar percentages of alloying ingredients. For example, it will be noted that in general the elongation is greatly improved, while the yield strength and tensile strength in both the annealed and cold rolled state shows an improvement over that of the related alloys. Similarly, an improvement in properties will be noted in the remaining portion of the composition range.

While the new alloy is most useful in wrought form, such as sheets, due to its formability char-

acteristics, it may also be suitably used in making castings, forgings, extruded forms, and the like. It is further pointed out that my new alloy is amenable to solution and precipitation heat treatments, which, accordingly, modify its properties.

My new alloys may be prepared by any of the methods usually employed for melting and alloying metals with magnesium, such as by adding the alloying materials singly or jointly to a bath of molten magnesium, which is preferably protected from oxidation by a suitable flux.

I claim:

1. A magnesium base alloy containing from 0.5 to 10 per cent of silver, from 1 to 15 per cent of cadmium, and from 0.1 to 10 per cent of zinc, the balance being magnesium.

2. A magnesium base alloy containing from 0.5 to 4 per cent of silver, from 6 to 12 per cent of cadmium, and from 0.5 to 4 per cent of zinc, the balance being magnesium.

3. A magnesium base alloy containing from 1 to 3 per cent of silver, from 6 to 12 per cent of cadmium, and from 0.5 to 4 per cent of zinc, the balance being magnesium.

JOHN C. McDONALD.